

1

3,288,627  
HEAT-SENSITIVE DIAZOTYPE MATERIAL  
COATED SHEET

Edward C. Bialczak, Mount Prospect, Ill., assignor to  
Addressograph - Multigraph Corporation, Cleveland,  
Ohio, a corporation of Delaware  
No Drawing. Filed Aug. 5, 1965, Ser. No. 477,594  
5 Claims. (Cl. 117—36.8)

This invention relates to heat-sensitive diazotype materials and to alkaline donor developers incorporated in such materials. More particularly, it relates to metallic dialkyldithiocarbamate-amine complexes and heat-sensitive diazotype materials coated with such complexes.

Heat-sensitive diazotype materials comprise a base member coated with a formulation containing a diazo compound and a coupling component with which the diazo compound reacts under proper conditions to form an azo dye which produces a visible image. In making a print, the diazotype material is exposed to light under a translucent master. In those areas of the diazotype material which are exposed to light, the light-sensitive diazo compound is at least partially destroyed, but is unaffected in the shaded areas. The print is then developed by heating the diazotype material and causing the alkaline donor developing agent to emit ammonia or an organic amine which produces the proper pH conditions for interaction of the diazo compound and the coupling component. These react to produce a dye image in the shaded area which corresponds to the graphic material on the master.

In conventional heat-sensitive diazotype materials the alkaline donor developer is commonly a urea or thiourea compound which on decomposition at elevated temperatures yields ammonia which induces the coupling reaction to form the azo dye. Urea and thiourea compounds produce diazotype materials having a relatively poor shelf life due to precoupling of the diazo compound and the coupling component at ambient temperatures. Other heat-sensitive diazotype materials which have longer shelf lives usually require higher temperatures to induce coupling. Generally, these temperatures are too high for office equipment and often they are so high that the diazo compound decomposes more rapidly than it reacts with the coupling component to form the azo dye. To cope with the problem of precoupling, increased amounts of acid have been used to stabilize the formulations, thus requiring increased amounts of alkaline donor to be incorporated into the formula to provide a sufficient source of ammonia to give a suitably dense image. For example, British Patent No. 909,491 proposes the use of certain types of acids which lose their acidity on heating and thereby reduce the required quantity of alkaline donor since at developing temperatures the acid is dissipated.

It is an object of this invention to provide heat-sensitive diazotype materials wherein the alkaline donor is stable at ambient temperature, decomposes to produce alkaline substances at relatively low temperature and does not contribute to precoupling. It is another object of this invention to provide heat-sensitive diazotype materials which form good prints and which have extended shelf life. It is a further object to provide alkaline donor materials for heat-sensitive diazotype materials which decompose at relatively low temperatures to provide alkaline materials which induce dye formation. These and other objects are apparent from and are achieved in accordance with the following disclosure.

In accordance with this invention it has been discovered that metallic dialkyldithiocarbamates form complexes with relatively strong organic amines. In these com-

2

plexes, which have the following general formula, one mole of metallic dialkyldithiocarbamate is combined with one mole of amine:



wherein  $R_1$ ,  $R_2$ ,  $R_3$  and  $R_4$  are lower alkyl radicals, Me is a metal (zinc, cadmium or tellurium) and Am is an organic amine. Among the alkyl radicals which  $R_1$ ,  $R_2$ ,  $R_3$  and  $R_4$  represent are methyl, ethyl, propyl, butyl, isobutyl and amyl radicals.

The organic amine, Am, can be any of a wide variety of non-aromatic amines containing 4 to 10 carbon atoms, inclusive. Primary aliphatic amines such as methylamine, ethylamine, n-butylamine, t-butylamine, hexylamine and decylamine are operative. Secondary aliphatic amines such as dimethylamine, methylethylamine, methyl-n-butylamine, and di-n-butylamine are also included in this group. Tertiary aliphatic amines which are operative include trimethylamine, triethylamine and the like.

The organic amine, Am, can also include alicyclic amines such as cyclohexylamine, N-methylcyclohexylamine, N-isopropylcyclohexylamine, N-butylcyclohexylamine, N-(2-cyanoethyl)cyclohexylamine, cyclobutylamine, N-methylcyclobutylamine, cyclopentylamine, N-ethylcyclopentylamine, cycloheptylamine, cyclooctylamine and related amines.

Hydroxyamines such as N-(2-hydroxyethyl)cyclohexylamine and N-(2-hydroxypropyl)cyclohexylamine are useful in this invention, as are diamines such as N-(2-aminoethyl)cyclohexylamine and N-(3-amino-propyl)cyclohexylamine. When diamines are combined with the metallic dialkyldithiocarbamate, they form complexes with both one mole and two moles of the metallic salts.

One important characteristic which determines the suitability of a particular amine as an alkaline donor when combined as a complex with a metallic dialkyldithiocarbamate is the pH of the complex in 10% aqueous mixture. Suitable amines form complexes which produce pH values not greater than 8.

The preferred amines in this invention are cyclohexylamine, t-butylamine and derivatives of cyclohexylamine such as N-(2-cyanoethyl)cyclohexylamine, N-(2-hydroxyethyl)cyclohexylamine and N-isopropylcyclohexylamine.

The complexes are readily produced by treating a slurry of a metallic dialkyldithiocarbamate in an inert solvent, such as benzene or other hydrocarbon liquid, with an equivalent quantity of the organic amine in the same solvent. The complex is insoluble in hydrocarbon solvents and can be readily isolated by filtration.

The metallic dialkyldithiocarbamate-amine complexes are dispersed in an inert solvent, such as toluene, in any conventional dispersion mill and applied directly to the substrate (e.g., paper) by roller coating or similar techniques in conjunction with an air knife or other suitable doctoring means. The alkaline donor coating can be applied as a precoat to the photosensitive coating or it can be applied over an existing photosensitive layer.

The metallic dialkyldithiocarbamate-amine complexes are water-insoluble, are stable at room temperature and dissociate in the temperature range from 100° to 150° C., releasing the amine. The latter raises the pH of the diazotype material and creates an environment in which the diazo compound can react with the coupling component to form an azo dye.

The light-sensitive diazo compounds which are useful in two-component diazotype systems can also be used to

advantage in thermally responsive diazotype materials. Examples of such compounds are the diazonium salts obtained by the diazotization of the following amines:

p-amino-N,N-diethylaniline  
 p-amino-N-ethylaniline  
 p-amino-N-ethyl-N- $\beta$ -hydroxyethylaniline  
 p-amino-N-methyl-N- $\beta$ -hydroxyethylaniline  
 p-amino-N,N-di( $\beta$ -hydroxyethyl)aniline  
 p-amino-m-ethoxy-N,N-diethylaniline  
 p-amino-N-ethyl-o-toluidine  
 p-amino-N-ethyl-m-toluidine  
 p-amino-N,N-diethyl-m-toluidine  
 p-amino-N-ethyl-N- $\beta$ -hydroxyethyl-m-toluidine  
 N-p-aminophenylmorpholine  
 1-amino-2,5-diethoxy-4-morpholinobenzene

The preferred diazo compound is the zinc chloride double salt of 4-morpholinobenzene diazonium chloride.

Generally, a number of coupling components may be employed. The preferred coupling component that may be employed to produce the dye image is 2,4-dihydroxy-naphthalene-6-sulfonic acid. Other known couplers may be employed such as resorcinol, acetoacetanilide, 4-chlororesorcinol and diacetooxyethylenediamine. It is, of course, desirable to select coupling components which have little tendency to react with the diazo compounds until the alkaline donor developer has released the amine upon being heated above about 100° C.

To prevent precoupling and premature dye formation, there can be added an acid component to keep the pH below the level required for coupling. Sulfonic acid derivatives, such as m-benzenedisulfonic acid, are employed as the preferred acid components. Other acids may be used to produce the desired pH such as:

|                      |               |
|----------------------|---------------|
| maleic acid          | oxalic acid   |
| malonic acid         | citric acid   |
| ethanesulfonic acid  | tartaric acid |
| benzenesulfonic acid | lactic acid   |

In addition to the acid components, there can be added to the diazo formulation certain heavy metal salts such as the sulfates of the zinc and cadmium. The inclusion of the heavy metal salts tends to prevent precoupling of the components at near room temperature.

By appropriate combinations of metallic dialkyldithiocarbamate-amine donors and acids, such as those listed above, it is possible to develop pH ranges between 5 and 12 which will induce reaction between any combination of diazo compound and coupling component.

The complexes of this invention, when exposed to heat, undergo dissociation to yield the corresponding amines which react with the free acid in the diazotype formulation. It is seen that the alkaline donors of this invention tend to lower the temperature to which the diazotype materials are subjected, simplify the equipment, produce more intense copy since the high temperatures which would degrade the diazo salts are avoided and increase the shelf life of diazotype materials.

When the metallic dialkyldithiocarbamate-amine complexes are applied to sheet materials in the production of diazotype materials, they are dispersed in fine particulate form in an organic solvent such as a hydrocarbon liquid (e.g., toluene) and the resulting suspension applied to the sheet material by conventional coating procedures. The complexes are usually present in the suspensions or dispersions at concentrations of 1% to 10% by weight, the range from 2% to 5% being preferred. The donor coating should be applied at a rate sufficient to afford in the range of 0.075 to 0.250 gram of complex per square foot of substrate, the preferred concentration being in the range of 0.1 to 0.125 gram of complex per square foot on a dry basis. After the solvent evaporates, the complexes form a thin coating of fine particles which can release an organic amine when activated by heat. It was found that the alkaline donor should be crystalline in

form so that it may be dispersed as particulate material in a solvent vehicle and deposited on the substrate as distinct particles.

In the photosensitive coating formulations for sheet materials, the amount of diazo compound is usually conventional. It generally constitutes 2% to 6% of the formulation with 4% being preferred. Equivalent quantities of coupling reagent are employed, following conventional practice. The coating formulations are applied in amounts 10 which will provide about 15 grams of diazo compound for 3,000 square feet of surface on a dry basis.

The base or substrate for the diazotype material can be paper or any other web or film material which is stable at 100°-150° C. Polyester films such as sold under the 15 trade names "Mylar" and "Kodar" are suitable film materials that may be used as stable substrates.

The invention is disclosed in more detail by the following examples which are provided for purposes of illustration only. It will be understood by those skilled in 20 the art that various combinations of diazo compounds, coupling components and alkaline donor developers can be used. It will also be understood that the amounts of ingredients in formulations and the operating conditions may be varied within this disclosure without departing 25 from the invention.

#### Example 1

Three moles of zinc dimethyldithiocarbamate (917 grams) are mixed with 5 liters of benzene. The mixture 30 is stirred for several hours forming a slurry. To the slurry there are gradually added 3 moles (297 grams) of cyclohexylamine in 350 milliliters of benzene which result in the formation of the zinc dimethyldithiocarbamate-cyclohexylamine complex. The complex is filtered off 35 under suction and washed with benzene to remove unreacted amine. The yield was 95% of product having a melting point in the range of 153° to 155° C. and a pH of a 10% complex-water mixture of 8.0.

The complex obtained from the above procedure is 40 used by applying it as a separate donor precoat to the base support for the thermal diazo sheet. A typical donor coating formulation is as follows:

| Parts by weight                                       |       |     |
|-------------------------------------------------------|-------|-----|
| 45 The amine - metallic alkyl dithiocarbamate complex | ----- | 2.5 |
| Toluene                                               | ----- | 100 |

The complex is dispersed in the toluene by any conventional dispersion type mill equipment and applied 50 directly to a paper substrate by the use of roller coating techniques in conjunction with an air knife.

On top of the donor coating there is applied photosensitive coating of which the following is a typical formula:

| Parts by weight                          |       |       |
|------------------------------------------|-------|-------|
| 55 Ingredient:                           | ----- | ----- |
| Water                                    | ----- | 100   |
| Citric acid                              | ----- | 2     |
| Thiourea                                 | ----- | 4     |
| 2,3-dihydroxynaphthalene-6-sulfonic acid | ----- | 6     |
| 60 Zinc sulfate                          | ----- | 4     |
| p-Diazo-N-ethyl-N-hydroxyethylaniline    | ----- | 1     |
| Silica particles (finely divided)        | ----- | 5     |
| Rice starch                              | ----- | 3     |
| Polyvinyl acetate emulsion               | ----- | 8     |

65 This diazotype paper is stable in storage, has a long shelf life and can be developed at relatively low temperature (110-120° C.).

#### Example 2

70 Three moles of cadmium dibutyldithiocarbamate suspended in 5 liters of toluene are treated with 3 moles of N-(2-hydroxyethyl)cyclohexylamine according to the procedure of Example 1. The resulting complex is collected on a filter, washed with toluene and dried. It is 75 dispersed in toluene (5 parts in 100 parts of toluene) and

the dispersion is coated on a dry diazotype paper coated with the photosensitive coating shown in Example 1. The resulting diazotype paper is stable in storage and can be developed at 115-130° C.

*Example 3*

Other metallic dialkyldithiocarbamate-amine complexes which are suitable in diazotype materials such as that described in Example 1 are listed below. These are prepared by the method of Example 1 by reacting a mole of the metallic dialkyldithiocarbamate with a mole of amine in an inert solvent such as benzene or toluene. In the case of diamines, two moles of the carbamate are reacted with one mole of the diamine. Each of these complexes dissociates at the temperature listed in the table below under "developing temperature" and releases amine which induces coupling of the diazo compound and the coupling component to form a dye which has the dye density listed in the table. In the table the developing temperature is measured on a hotplate device and represents the temperature at which the amine is released.

|                                                                  | Dye Density | Developing Temp., °C. |
|------------------------------------------------------------------|-------------|-----------------------|
| Zinc dimethyldithiocarbamate cyclohexylamine                     | 1.1         | 115                   |
| Zinc diethyldithiocarbamate cyclohexylamine                      | .83         | 105                   |
| Zinc dibutylidithiocarbamate cyclohexylamine                     | 1.1         | 115                   |
| Zinc diethyldithiocarbamate tert-butylamine                      | 1.04        | 115                   |
| Zinc diethyldithiocarbamate N-(2-hydroxyethyl) cyclohexylamine   | 1.02        | 130                   |
| Zinc diethyldithiocarbamate N-(2-cyanoethyl) cyclohexylamine     | 1.30        | 138                   |
| Zinc diethyldithiocarbamate N-isopropylcyclohexylamine           | .87         | 138                   |
| Zinc dimethyldithiocarbamate N-(2-hydroxyethyl)cyclohexylamine   | .90         | 140                   |
| Zinc dimethyldithiocarbamate tert-butylamine                     | .90         | 145                   |
| Zinc dimethyldithiocarbamate N-(2-cyanoethyl)cyclohexylamine     | .90         | 152                   |
| Zinc dibutylidithiocarbamate N-(2-cyanoethyl)cyclohexylamine     | .73         | 125                   |
| Zinc dimethyldithiocarbamate N-isopropylcyclohexylamine          | .85         | 145                   |
| Zinc dimethyldithiocarbamate N-ethylcyclohexylamine              | .75         | 145                   |
| Zinc dimethyldithiocarbamate N-(3-aminopropyl)cyclohexylamine    | .79         | 145                   |
| Dilzinc dimethyldithiocarbamate N-(3-aminopropyl)cyclohexylamine | .82         | 145                   |
| Zinc dibutylidithiocarbamate N-isopropylcyclohexylamine          | .43         | 138                   |
| Cadmium diethyldithiocarbamate cyclohexylamine                   | .8          | 105                   |
| Cadmium dimethyldithiocarbamate cyclohexylamine                  | 1.0         | 125                   |
| Tellurium diethyldithiocarbamate cyclohexylamine                 | 1.04        | 115                   |

I claim:

1. A heat-sensitive diazotype material comprising a base sheet coated with a diazo compound, a coupling component and an alkaline donor metallic dialkyldithiocarbamate-amine complex, wherein the metal is selected from the group consisting of zinc, cadmium and tellurium, the alkyl radicals contain 1 to 5 carbon atoms, inclusive, and the amine is selected from the group consisting of aliphatic and alicyclic amines containing 4 to 10 carbon atoms, inclusive.
- 5 2. A heat-sensitive diazotype material comprising a base sheet coated with a diazo compound, a coupling component and an alkaline donor metallic dialkyldithiocarbamate-amine complex as defined by claim 1 wherein the amine is an aliphatic amine containing 4 to 10 carbon atoms, inclusive.
- 10 3. A heat-sensitive diazotype material comprising a base sheet coated with a diazo compound, a coupling component and an alkaline donor metallic dialkyldithiocarbamate-amine complex as defined by claim 1 wherein the amine is an alicyclic amine containing 4 to 10 carbon atoms, inclusive.
- 15 4. A heat-sensitive diazotype material comprising a base sheet coated with a diazo compound, a coupling component and an alkaline donor zinc dialkyldithiocarbamate-cyclohexylamine complex, wherein the alkyl radicals contain 1 to 5 carbon atoms, inclusive.
- 20 5. A heat-sensitive diazotype material comprising a base sheet coated with a diazo compound, a coupling component and an alkaline donor zinc dimethyldithiocarbamate-cyclohexylamine complex.

References Cited by the Examiner

UNITED STATES PATENTS

- |    |           |                           |           |
|----|-----------|---------------------------|-----------|
| 35 | 2,732,299 | 1/1956 Morrison           | 117-36.8  |
|    | 2,967,784 | 1/1961 Newman et al.      | 117-36.8  |
|    | 2,995,465 | 8/1961 Richey             | 117-36.8  |
|    | 2,999,035 | 9/1961 Sahler             | 117-36.8  |
| 40 | 3,057,895 | 10/1962 Marblehead et al. | 260-429.9 |
|    | 3,076,707 | 2/1963 Lawton et al.      | 117-36.8  |
|    | 3,149,990 | 9/1964 Coles et al.       | 117-36.8  |
|    | 3,157,526 | 11/1964 Johnson et al.    | 117-36.8  |
|    | 3,177,233 | 4/1965 Calhoun            | 260-429.9 |
| 45 | 3,185,585 | 5/1965 Baumann et al.     | 117-36.8  |
| 50 | 3,191,030 | 6/1965 Huett et al.       | 117-36.8  |

OTHER REFERENCES

- Kosar: "Thermal Development of Diazo Papers," "Photographic Science and Engineering," vol. 5, No. 4, July-August 1961, pp. 239-243.

MURRAY KATZ, Primary Examiner.